

## UNITED STATES PATENT OFFICE.

ALFRED L. BOEGEHOOLD, OF DETROIT, MICHIGAN, ASSIGNOR TO GENERAL MOTORS RESEARCH CORPORATION, OF DETROIT, MICHIGAN, A CORPORATION OF DELAWARE.

## MALLEABLE IRON ALLOY.

No Drawing.

Application filed March 14, 1927. Serial No. 175,435.

It is an object of this invention to produce malleable iron castings of any size and shape by (1) pouring a molten mixture of iron, carbon and a graphitizing agent, (that is an agent capable of decomposing combined iron and carbon into graphite and iron) to which has been added an alloying ingredient having the property of preventing the formation of flake carbon during the period of solidification and cooling, and (2) thereafter heat treating the casting until it becomes malleable.

The process of making malleable iron castings according to the heretofore usual practice consists in pouring into an ordinary green sand mold molten iron having a silicon content low enough to prevent the formation of carbon in flake form in the mold, then removing the casting and annealing it by subjecting it to heat treatment continuing for a period of about 110 hours. The heat treatment consists in first, raising the temperature of the casting and its environment to about 1600° to 1700° F., requiring about 30 hours, second, maintaining the temperature of about 1600° to 1700° F., for about 40 hours; third, slowly cooling the casting to just below the lower critical temperature (which is approximately 1340° F.) and holding this temperature for about 35 hours; and, fourth, cooling to a temperature low enough to permit handling, which requires about 5 hours,—a total period of about 110 hours, which cannot be very much reduced.

Iron commonly used in the customary process of making malleable castings has a silicon content of from .90% to 1.10%; it cannot run much above 1.30% in the described process of the prior art, in which the carbon content is usually 2.40 to 2.60%, without danger of precipitating carbon in flake form, which would destroy the property of malleability. It is generally understood that the quantity of carbon plus silicon in the mix employed in practicing the ordinary process must not substantially exceed 3.75%, if iron having the white fracture characteristic of castings ca-

pable of being malleabilized is to be produced.

In view of the necessarily high cost of malleable iron production by the described standard process, due to the long period of heat treatment necessary, I have sought to develop a process of making iron products, cast in molds, that may be annealed in a much shorter time; that may approximate or equal the standard malleable iron product in tensile strength, malleability and ductility, and equal or exceed it in machineability.

In Patent No. 1,591,598, issued to Harry M. Williams and myself on July 6th, 1926, is described and claimed a process for the production of malleable castings in which the desired shortening of the annealing time is accomplished by the employment of larger proportions of temper carbon forming or graphitizing agent, such as silicon, than could be employed in said customary process; and, to prevent precipitation of the carbon in flake form during casting, owing to the presence of the added quantity of this ingredient, the iron is cast in chill molds, preferably permanent metallic molds, so that it will cool as rapidly as possible. Satisfactory malleables can be produced by this process.

However, the permanent mold process is not applicable to all shapes and sizes of castings; wherefore I have sought to develop a process of more general application, useful for the production of malleable castings of a wide range of shape and size.

It has also been proposed heretofore to shorten the annealing time of malleables by employing a lower percentage of carbon in the mix than has been used in the aforesaid usual process, this lower carbon percentage permitting an increase in the percentage of the graphitizing agent, such as silicon, with a consequent shortening of the annealing time. I have found that where this process (which may be here termed the low carbon process) is employed there is a limit to the sum total percentage of silicon and carbon that can be included in the mix, which total

must not be exceeded if precipitation of flake carbon while the casting is solidifying in the mold and cooling is to be avoided. This process is subject to the disadvantage that 5 owing to the low proportion of carbon present the metal lacks fluidity, at least under some conditions,—that is, its melting point is raised, rendering it more difficult and expensive to work,—and furthermore it is limited to the production of malleable castings 10 of relatively thin cross section.

In attacking the problem to be solved by this process I have been governed by the following limiting conditions:

15 (1) Precipitation of flake graphite during solidification of the casting must be avoided;

(2) A sufficient quantity of graphitizing agent to hasten annealing, as compared with the period of time required by said customary 20 process, must be present;

(3) The casting metal must have a low melting point and high fluidity in order to economize in time and fuel when melting, prolong the life of the refractories in the 25 melting receptacle and permit the metal to fill the interstices of the mold;

(4) The process must be adapted to produce castings in ordinary sand molds, although preferably also equally well adapted 30 to the use of permanent metallic molds;

(5) The process must produce castings showing a white fracture independently of the thickness of the casting.

I have found that it is possible to satisfy 35 all of the foregoing named conditions to a greater or less extent by adding to a suitable casting composition of iron, carbon and silicon or the like a suitable quantity of an ingredient having the property of obstructing 40 the formation of flake graphite, which may be one of several metals capable of alloying with iron.

According to the invention that is the subject of this application I employ a composition 45 of molten metal to be cast consisting (except for impurities commonly present in cast iron) of iron, carbon, and a graphitizing agent, preferably silicon, wherein the proportion of graphitizing agent is higher than 50 can be used in the aforesaid customary process and wherein the total proportion of carbon and silicon may be considerably higher; and also an additional metallic ingredient that has the aforesaid property of preventing 55 or obstructing the precipitation of graphite in flake form by the action of the graphitizing agent. The percentage of carbon should preferably be high enough to impart a low melting point and high degree of fluidity to 60 the casting metal; the percentage of silicon or equivalent graphitizing agent can be made high enough to enable the casting to be annealed in a short period of time; by reason of the presence of the said additional metal-

lic ingredient the flake graphite precipitating tendency of the large proportion of silicon or the like present in the casting metal can be prevented during solidification and cooling of the casting and, in addition, a casting that will show a white fracture can 70 be made independent of shape or size of cross section. Castings poured from molten mixtures as described can be rendered malleable by a relatively short heat treating or annealing 75

Among many substances tested it has been found that any one of the metals molybdenum, vanadium, nickel or copper, when introduced in suitable quantity in a cast iron mixture containing a proper proportion of 80 silicon and carbon, has proved efficacious in preventing formation of flake graphite during solidification and subsequent cooling of castings poured from the mixture. Of the several elements that prevent or retard formation of flake graphite one may have also an effect of retarding the action of silicon in breaking down iron carbide to form temper carbon during annealing or heat treatment 85 of the casting, while another may assist this 90 action. The characteristic action of the element selected with respect to the decomposition of iron carbide may affect the proportions of silicon or the like required in the mix. 95

It has also been ascertained that the addition to the mix or casting metal of a small proportion of metal having the said property of preventing or obstructing formation of flake graphite makes it possible to use a 100 large proportion of the graphitizing or carbon precipitating agent without that formation of flake graphite which would occur if said metal had not been added.

In making white iron castings by sand mold processes, using a mix consisting of iron, silicon and carbon the sum of silicon and carbon cannot substantially exceed 3.75% of the mix, as heretofore stated. But, in an iron-silicon-carbon mixture containing in addition .50% molybdenum, it is possible to include 2.59% carbon and 1.80% silicon (carbon plus silicon=4.39%) without producing a casting showing a grey fracture; a molybdenum content of .50% with 2.48% carbon and 2.30% silicon (carbon plus silicon=4.78%) also gives a casting without grey fracture. The addition of the .50% of molybdenum increases the amount of silicon that can be employed without imparting the characteristics of grey iron to the casting. Iron casting showing the best physical properties thus far obtained by this process have been poured from an iron mix containing 2.27% carbon, 1.50% silicon (carbon plus silicon=3.77%) and .50% molybdenum. Tests of malleable castings made from this alloy showed a tensile strength of 71800 pounds 115 120 125

per sq. inch, and an elongation of 10.5%. Molybdenum may be introduced in the form of ferromolybdenum or molyte (a compound of molybdenum and calcium silicide).

5 Experiments with nickel as an alloying ingredient have proven that an iron mix containing 2.11% carbon and 1.77% silicon (carbon plus silicon=3.88%) and a nickel content of 1.33% will afford a casting of white 10 iron in spite of the fact that nickel itself is considered a graphitizing agent. The effect of nickel as a graphitizing agent here is more apparent at the annealing temperatures than at the higher temperatures in the mold 15 during solidification. Annealed castings made from the described nickel-containing mix showed upon test a tensile strength of 62000 pounds per square inch and an elongation of 4.5%.

20 By introducing .25% vanadium into a mixture of iron casting-metal it is possible to use 2.26% of carbon and 1.81% of silicon (carbon plus silicon=4.07%), and still obtain a casting having a white fracture. Higher percentages 25 of vanadium although giving a white iron casting appear to slow the annealing process. An annealed casting made of iron with 2.05% carbon and 1.81% silicon (carbon plus silicon=3.86%) and less than .25% 30 vanadium has shown a tensile strength of 65000 pounds per square inch and an elongation of 10%.

The introduction of copper into the casting metal permits, as does nickel, a much higher 35 carbon plus silicon content than could be used to produce a casting giving a white fracture in the absence of copper. Using .50% copper, 2.30% carbon and 1.97% silicon, (carbon plus silicon=4.27%) castings have been 40 obtained the fractures of which are white. However, annealed castings made from copper-containing mixtures do not possess as high tensile strength and elongation as castings containing the other alloying ingredients 45 mentioned.

The time required for annealing castings made by the process of this application is very much less than that required by the standard process of making malleable iron. 50 A small number of castings containing alloying metals mentioned above were heat treated 19½ hours in an open furnace, not packed in boxes, and were tested for physical properties with the results stated. In these tests 55 1½ hours were required to heat the castings to annealing temperature, about 15½ hours to anneal (i. e. to precipitate the combined carbon in the form of temper carbon) while maintaining the annealing temperature of 60 about 1650° F., and about 2½ hours to cool the castings to 1150° F., when they were removed from the heating apparatus.

It has been found that when the described 65 alloy casting-metal containing one of the metals for obstructing formation of flake graph-

ite is poured into a mold, the rate of cooling in the mold is not a highly important factor in producing a casting having a white fracture, as it is in processes involving casting in permanent or other chill molds.

70

Whereas, also, castings made of ordinary iron of proper analysis to produce small malleable casting in prior known processes might show a white fracture in a casting of one inch section, a two inch section might 75 show a grey fracture. But a casting made from one of the alloy compositions according to this invention of analysis proper to show a white fracture in a ¾ inch or 1 inch casting will show a white fracture also if the 80 casting be of 2 inch or larger section. It will be obvious that this property is of very great advantage in the art of making malleables.

80

There are graphitizing or temper carbon forming elements other than silicon; for example, nickel as already mentioned, copper, titanium, zirconium and aluminum. Aluminum for instance may be substituted for silicon with substantially similar effects with respect to precipitation of carbon in temper carbon 90 form and obstruction of formation of flake carbon. As, however, the presence of aluminum confers certain undesirable properties upon the metal in molten condition, which make it undesirable for casting, it is less suitable than silicon for use as a graphitizing 95 agent. Where the graphitizing agent is also a metal that obstructs formation of flake graphite it may be possible to do without a separate graphitizing agent, or to use a 100 smaller proportion of a separate graphitizing agent. But the quantity of alloying metal to be used under these circumstances is likely to be so large as to confer undesirable properties upon the casting.

105

The substances usually present as impurities in mixtures used for making malleable iron castings are sulphur, phosphorus and manganese. In the casting mixture utilized in the process of this application the quantity 110 of sulphur can be as high as in any form of commercial malleable now known, but according to my experience it should be kept preferably below .085%. Phosphorous should preferably be below .20%, and manganese below 115 .50%. A manganese content above .50% renders annealing more difficult. A mixture containing .45% manganese works satisfactorily in this process.

110

The carbon content of a mixture suitable 120 for use in this process should be high enough to give a low melting point and high fluidity. It should not therefore be substantially less than 2.00%. It should not be so high as to weaken the texture of the annealed casting, and I consider that more than 2.75% carbon is too high.

120

The silicon content should be high enough 125 to form temper carbon during a short annealing period but not high enough to form flake

130

graphite during solidification. These conditions place the low limit of silicon at about 1.80% and the high limit at about 2.50%.

It should be apprehended that the proportion of either the silicon or carbon ingredient that may be used successfully in this process depends to some extent on the proportion of the other. In general, if the percentage of silicon is near the higher limit, the percentage 10 of carbon ought to be lower than if the silicon content were nearer the lower limit, and vice versa. My experience indicates that the sum total of silicon and carbon in the casting composition should not exceed 4.80%, more or 15 less. In any event the relative proportions of carbon and silicon within the ranges mentioned should not be such as to impart the characteristics of grey iron to the casting; the castings should have a white fracture.

20 The limits of the percentage of metal used as an obstructor of flake graphite formation are theoretically quite wide. Ordinarily as little as may be required to produce the desired result should be used. Otherwise the 25 cost (particularly when using molybdenum or vanadium) would probably be prohibitive; also, other characteristics that are undesirable might be imparted to the alloy. Too much vanadium, for example, tends to 30 prevent silicon from precipitating the carbon during the annealing operation, while too much copper tends to form globules of copper in the iron during solidification in the mold,—that is, a too high copper content will not 35 wholly alloy with the iron. The permissible percentage of copper depends to an extent on the percentages of silicon and carbon present. The graphitizing properties of nickel and copper constitute another limiting factor to 40 the quantity of nickel or copper that can be used, which must be less than that which causes formation of flake graphite.

A principal feature of this process is the 45 use of a relatively larger proportion of silicon, or similar graphitizing agent, than in the customary process, together with an element alloyable with iron that obstructs formation of flake graphite. Although the total content of carbon plus silicon is generally 50 larger than in the usual practice it is not necessarily so, but the silicon content should be larger; and this permits the use of sufficient carbon to provide a low melting point casting composition even though the total of 55 carbon and silicon be considerably larger than in standard practice.

The metal to be cast may be melted in a suitable melting furnace such as an air furnace, electric furnace, or cupola used in connection with an electric furnace.

60 The castings may be annealed at the usual annealing temperature (around 1600° F.) and may be heated gradually although rapidly to this temperature and after maintaining it

for a brief period gradually though rapidly 65 cooled. For annealing purposes an annealing furnace of the type in which the article to be annealed may be carried through it in conveyors or cars may be used. A tunnel kiln of the Dressler type is well adapted for the 70 purpose. As heretofore indicated satisfactory results have been achieved after heat treating for 19½ hours under the conditions heretofore stated. In commercial practice, where a large number or large mass of castings are 75 placed in the annealing furnace it would require about 50 hours, more or less, because of the time necessarily consumed in heating all parts to the annealing temperature and permitting cooling to a temperature at which the 80 castings can be handled. The time during which the annealing temperature should be maintained would be about 15 or 16 hours, the remainder of the 50 hours being required to bring the castings up to annealing temperature and thereafter to cool them.

In using the term "white iron casting" I mean a carbon containing iron free of carbon in flake form that characterizes ordinary grey iron castings. I do not intend the term 90 "white iron" to exclude annealable iron castings that may contain some nodular or temper carbon but contain substantially no flake carbon.

Annealed castings produced by the process 95 of this application show the same microstructure that characterizes standard malleable castings made in the heretofore customary manner, and appear in all respects to be adapted for use wherever malleable castings 100 are needed.

While in order to comply with the statutes, I have set forth the principle of my invention and have given several analyses of casting metals for use in practicing it, including that 105 one which I have thus far found to be most suitable, it will be understood that the principle may be applied by the skilled metallurgist with other analyses and that I do not intend to be limited to examples given except 110 as indicated in the appended claims.

What I claim is:

1. An annealable white iron casting free from flake graphite comprising iron, carbon, a graphitizing agent capable of promoting 115 formation of temper carbon during annealing, and a suitable proportion of a metallic ingredient having the property of obstructing formation of flake graphite during solidification of the casting.

2. An annealable white iron casting as defined in claim 1, comprising from 1.30% to 2.50% of silicon, and a sum total of silicon plus carbon not substantially over 4.80%.

3. An annealable white iron casting as defined in claim 1, comprising from 2% to 2.75% of carbon, and a sum total of silicon plus carbon not substantially over 4.80%.

4. An annealable white iron casting as defined in claim 1, comprising from 1.30% to 2.50% of silicon and from 2% to 2.75% of carbon.
5. An annealable white iron casting as defined in claim 1, in which the metallic ingredient capable of obstructing the formation of flake graphite during solidification of the casting is totally alloyed with the iron.
- 0 6. An annealable white iron casting as defined in claim 1, in which the metallic ingredient capable of obstructing formation of flake graphite during solidification of the casting is molybdenum.
7. An annealable white iron casting free from flake graphite consisting of iron, carbon and silicon, and a small proportion of molybdenum alloyed with the iron.
8. An annealable white iron casting as defined in claim 7 containing iron, about 2.75% carbon, about 1.80% silicon and about .50% molybdenum.

In testimony whereof I affix my signature.  
ALFRED L. BOEGEHOOLD.